



US007603755B2

(12) **United States Patent**  
**Gordon**

(10) **Patent No.:** **US 7,603,755 B2**  
(45) **Date of Patent:** **Oct. 20, 2009**

(54) **METHOD OF PRODUCING A TWILL WEAVE FABRIC WITH A SATIN FACE**

(75) Inventor: **Dean Gordon**, Hickory Grove, SC (US)

(73) Assignee: **Northeast Textiles, Inc.**, Bowling Green, SC (US)

(\*) Notice: Subject to any disclaimer, the term of this patent is extended or adjusted under 35 U.S.C. 154(b) by 506 days.

(21) Appl. No.: **11/511,967**

(22) Filed: **Aug. 29, 2006**

(65) **Prior Publication Data**

US 2008/0052884 A1 Mar. 6, 2008

(51) **Int. Cl.**

**D06C 27/00** (2006.01)

(52) **U.S. Cl.** **26/28; 28/163; 28/165**

(58) **Field of Classification Search** **26/28, 26/27, 51, 52, 89, 92, 29 R, 30; 28/163, 28/165, 140; 139/1 R, 291 R, 307, 383 R; 451/54, 57**

See application file for complete search history.

(56)

**References Cited**

**U.S. PATENT DOCUMENTS**

3,523,346 A \* 8/1970 Bolen et al. .... 28/163  
3,973,359 A \* 8/1976 Spencer et al. .... 451/183  
4,103,054 A \* 7/1978 Okamoto et al. .... 428/91  
4,145,467 A \* 3/1979 Malik .... 26/29 R  
4,316,928 A \* 2/1982 Otto .... 442/195  
5,815,896 A \* 10/1998 Dischler .... 26/28  
6,233,795 B1 \* 5/2001 Dischler .... 26/28  
6,242,370 B1 \* 6/2001 Dischler .... 26/28  
7,055,227 B2 \* 6/2006 Love et al. .... 28/167  
2003/0154580 A1 \* 8/2003 Overcash et al. .... 26/27  
2004/0229538 A1 \* 11/2004 Love et al. .... 442/182  
2008/0227351 A1 \* 9/2008 Park et al. .... 442/192

\* cited by examiner

*Primary Examiner*—Amy B Vanatta

(74) *Attorney, Agent, or Firm*—J. Bennett Mullinax, LLC

(57)

**ABSTRACT**

A method of forming a fabric is provided. The method includes the step of providing a plurality of yarn and batching the yarn on an A-frame so that the fabric is formed with a width greater than 102 inches and with a twill weave with a satin face. Also included is the step of passing the fabric across a plurality of rolls that have a rough surface and that apply compression to the fabric. The steps of applying fabric to a tenter frame and heating of the fabric is also included. The present invention also provides for a fabric in certain exemplary embodiments.

**16 Claims, 2 Drawing Sheets**





FIG. 1



FIG. 2



FIG. 3

**METHOD OF PRODUCING A TWILL WEAVE  
FABRIC WITH A SATIN FACE**

**FIELD OF THE INVENTION**

The present invention relates generally to a method of producing a twill weave fabric that has a satin face. More particularly, the present application involves a method of producing a 3/1 or 4/1 twill weave fabric with a satin face that has a large width which permits the seamless production of draperies, comforters, curtains, and other large finished fabric articles.

**BACKGROUND**

Fabric is a man-made flexible material composed of a network of artificial or natural fibers. The network of fibers can be made through the process of weaving or knitting. Fabrics can be constructed in a variety of manners in order to achieve various properties. For example, when incorporated into curtains the fabric can be designed in order to be opaque to block outside light. Further, the fabric can be constructed to have a high quality hand feel for items such as a bed comforter which improves the comfort and feel of the comforter. Consumers perceive a fabric that has "good hand" properties as a higher quality product and, thus, it is an important consideration in the consumer's selection of a fabric.

A weave pattern of the fabric includes a plurality of yarn pieces that are parallel to one another and are known as warp yarns. The warp yarns are usually oriented perpendicular to another plurality of parallel yarns known as weft yarns. The warp and weft yarns overlay and underlay one another in particular patterns in order to result in the weave pattern of the fabric. The weave pattern repeats throughout the fabric, and the ends per weave repeat is the number of warp yarns that are present in one repeating pattern.

Fabric that has a twill weave is generally structured so that two or three warp yarns are positioned over a weft yarn. Further, one or two warp yarns are positioned under the respective weft yarn. Fabrics with a twill weave are generally more wrinkle resistant, more durable, and are more resistant to showing soil than fabrics with a plain weave. Additionally, twill weave fabrics have fewer interlacings, are more pliable and have better hand feel than plain weave fabrics. Satin weave fabrics typically have a structure in which interlacings float over four or more yarns. As such, satin weave fabrics usually have floats that may be 3/1, 4/1, 7/1 and 11/1. These types of fabrics are typically flat with a smooth, lustrous surface.

Fabrics are treated during the production process in order to achieve or enhance various properties. For example, the fabric may be sanded, heated, stretched or treated with a chemical agent. Fabric for use in curtains, for instance, can be selected as a 3/1 or 4/1 twill weave fabric with a satin face and may be treated during the production process with an agent for inducing soil release. Such fabrics can have variously designed print patterns imparted thereon and once formed can be sewn together to be used in a curtain of a desired length. Formation of curtains or bed spreads in this manner may be problematic in that a great deal of care and time must be used in order to make the print patterns line up between successive fabric pieces. Additionally, the presence of seam lines in the final product may be undesirable to the end user. It is currently not feasible to produce fabrics in greater widths to alleviate these problems as roller oscillation occurs with fabrics of greater width resulting in uneven surface finishes of the final product.

As such, there remains room for variation and improvement within the art.

**SUMMARY**

Various features and advantages of the invention will be set forth in part in the following description, or may be obvious from the description, or may be learned from practice of the invention.

One aspect of the present invention provides for a method of finishing a fabric that has a twill weave with a satin face. The method includes the steps of providing a fabric that has a width from 102 to 131 inches. Additional steps include sewing and batching the fabric on an A-frame. The fabric is passed at a speed of 20 yards per minute with a first roll that has a 120 grit sand paper surface and that rotates in a counter clockwise direction. The first roll applies 3 inches of compression to the fabric. The fabric engages a second roll that has a 100 grit sand paper surface and that rotates in a clockwise direction. The second roll applies 7 inches of compression to the fabric. The fabric also engages a third roll that has a 100 grit sand paper surface and that rotates in the clockwise direction. The third roll applies 7 inches of compression to the fabric. The fabric also engages a fourth roll that has a 120 grit sand paper surface and that rotates in a counterclockwise direction. The fourth roll applies 5 inches of compression to the fabric. The method also includes applying the fabric to a tenter frame and stretching the fabric by 2% of the fabric's relaxed length. The fabric is moved at a speed from 15 to 35 yards per minute. Another step involves applying an agent to the fabric to improve pilling properties of the fabric. A further step includes heating of the fabric to a temperature of 385 degrees Fahrenheit.

Another aspect of the present invention is found in a method of forming a fabric that includes the step of providing a plurality of yarn. The method also includes batching the yarn on an A-frame so that the fabric is formed with a width greater than 102 inches and with a twill weave with a satin face. Also included in the method is the step of passing the fabric across a plurality of rolls that have a rough surface in which the rolls apply compression to the fabric. Additional steps involve applying the fabric to a tenter frame and heating of the fabric.

A further aspect of the present invention is found in a method as immediately discussed that further has the step of sanding the fabric at a speed of 20 yards per minute.

An additional aspect of the present invention exists in a method as previously discussed in which the passing step includes the passing of the fabric across a first roll that has a 120 grit sand paper surface and that rotates in a first direction. The first roll applies at least 3 inches of compression to the fabric. The passing step also involves passing the fabric across a second roll that has a 100 grit sand paper surface and that rotates in a second direction. The second roll applies at least 7 inches of compression to the fabric. Also included in the passing step is the action of passing the fabric across a third roll that has a 100 grit sand paper surface and that rotates in the second direction. The third roll applies at least 7 inches of compression to the fabric. Also included in the passing step is the passing of the fabric across a fourth roll that has a 120 grit sand paper surface and that rotates in the first direction. The fourth roll applies at least 5 inches of compression to the fabric.

Another aspect of the present invention is found in a method as previously discussed in which the applying step includes stretching of the fabric by 2% of the fabric's relaxed length.

The present invention provides for in another aspect a method as previously discussed that further includes the application of an agent to the fabric. The agent acts to improve the soil release and pilling properties of the fabric.

Another aspect of the present invention is found in a method as discussed above in which the fabric is formed in the sewing and batching step so as to have a float of 3/1.

Another aspect of the present invention exists in a method as previously mentioned in which the fabric is formed in the sewing and batching step so as to have a float of 4/1.

An additional aspect of the present invention is found in a method mentioned prior in which the width of the fabric is 124 inches.

Also provided in another aspect of the present invention is a fabric that has a plurality of yarns that are formed into a 3/1 or a 4/1 twill weave face with a satin face. The fabric has at least 110 ends that are single-ply. The fabric has a width of at least 102 inches and is seamless.

An additional aspect exists as previously mentioned in which the width of the fabric is 124 inches.

The present invention also provides for a method of forming a fabric that includes the step of providing a plurality of polyester yarn. The method also involves sewing and batching the yarn on an A-frame so that the fabric is formed with a width from 102 inches to 131 inches and with a 3/1 or 4/1 twill weave with a satin face. Sanding of the fabric is also employed at a speed of at least 20 yards per minute. Another step involves passing the fabric across a plurality of rolls that have a sand paper surface in which the rolls apply compression to the fabric. The fabric is further applied to a tenter frame so that the fabric is stretched by at least 2% of its relaxed length. Another step involves treating the fabric with an agent to improve pilling properties of the fabric. Further, the fabric is heated in an additional step to a temperature of at least 385 degrees Fahrenheit.

Another aspect of the present invention resides in a method as immediately discussed in which the passing step includes passing the fabric across a first roll that has a 120 grit sand paper surface that will rotate in a first direction. The first roll applies at least 3 inches of compression to the fabric. The passing step also includes passing of the fabric across a second roll that has a 100 grit sand paper surface and that rotates in a second direction. The second roll applies at least 7 inches of compression to the fabric. The fabric is further passed in the passing step across a third roll that has a 100 grit sand paper surface and that rotates in the second direction. The third roll applies at least 7 inches of compression to the fabric. The passing step also includes passing of the fabric across a fourth roll that has a 120 grit sand paper surface and that rotates in the first direction. The fourth roll applies at least 5 inches of compression to the fabric.

An additional aspect of the present invention is found in a method as previously discussed that further includes the step of moving the fabric at a speed from 15 to 35 yards per minute.

These and other features, aspects and advantages of the present invention will become better understood with reference to the following description and appended claims. The accompanying drawings, which are incorporated in and constitute part of this specification, illustrate embodiments of the invention and, together with the description, serve to explain the principles of the invention.

skill in the art, is set forth more particularly in the remainder of the specification, which makes reference to the appended Figs. in which:

FIG. 1 is a perspective view of a fabric in accordance with one exemplary embodiment of the present invention.

FIG. 2 is an enlarged plan view of circle A in FIG. 1 that shows the weave pattern of the fabric.

FIG. 3 is an enlarged plan view of the weave pattern of the fabric in accordance with an alternative exemplary embodiment of the present invention.

Repeat use of reference characters in the present specification and drawings is intended to represent the same or analogous features or elements of the invention.

#### DETAILED DESCRIPTION OF REPRESENTATIVE EMBODIMENTS

Reference will now be made in detail to embodiments of the invention, one or more examples of which are illustrated in the drawings. Each example is provided by way of explanation of the invention, and not meant as a limitation of the invention. For example, features illustrated or described as part of one embodiment can be used with another embodiment to yield still a third embodiment. It is intended that the present invention include these and other modifications and variations.

It is to be understood that the ranges mentioned herein include all ranges located within the prescribed range. As such, all ranges mentioned herein include all sub-ranges included in the mentioned ranges. For instance, a range from 100-200 also includes ranges from 110-150, 170-190, and 153-162. Further, all limits mentioned herein include all other limits included in the mentioned limits. For instance, a limit of up to 7 also includes a limit of up to 5, up to 3, and up to 4.5.

The present invention provides for a fabric and a method of forming a fabric that has a twill weave with a satin face. The fabric can be formed with a float of 3/1 or 4/1 and may have a width of at least 102 inches, and preferably about 124 inches. Other embodiments exist in which the width may be from 102 inches to 131 inches.

The method, in accordance with one exemplary embodiment of the present invention, involves weaving on a loom a polyester warp yarn having about 140-150 denier with about 36-100 filaments in a single-ply form, although two-ply is possible in other embodiments. Also woven is a polyester two-ply yarn of about 140-150 denier weft yarn with between about 36-110 filaments and a pick count of 55. The fabric is woven at a width of about 124 inches. The yarn can be made from either plain polyester or may be made of 100% fire retardant polyester. Alternatively, the yarn can be made with a blend of fire retardant polyester and plain polyester, which is useful for heat transfer printing of fabrics.

The yarn may be put through a sewing and batching process on an A-frame. Here, the yarn is formed into a fabric such as a 3/1 or 4/1 twill weave that has a satin face. The ends of the fabric are single ply in one embodiment. Further, 110 or more ends may be present in accordance with other exemplary embodiments. The warp yarns of the fabric are oriented in the length-wise direction and extend in the machine direction during subsequent processing. The weft yarns of the fabric extend in the cross-direction and hence along the width of the fabric. The width of the fabric may be from 102 to 131 inches in accordance with certain exemplary embodiments. In accordance with one exemplary embodiment, the width of the fabric is 124 inches.

Following weaving, the fabric is then typically taken to a second location and subjected to various procedures such as

#### BRIEF DESCRIPTION OF THE DRAWINGS

A full and enabling disclosure of the present invention, including the best mode thereof, directed to one of ordinary

finishing or preparation steps using conventional protocols. In such procedures the fabric may be, for example, dyed and/or treated so as to be fire retardant. Thereafter, in a subsequent treatment step, the fabric is sanded at a rate of 20 yards per minute. However, it is to be understood that sanding at different rates may be employed in other embodiments. For example, the fabric can be sanded at a rate up to 30 yards per minute or may be sanded at a rate up to 15 yards per minute. The longer floats of the fabric result in ends that are not tied down and hence sand more evenly to achieve a more desirable fabric finish.

Sanding is accomplished by passing the fabric surface(s) over a plurality of rollers. The rollers can be provided with a rough surface for treating the fabric. For example, the rollers can have sand paper surfaces in one embodiment. In accordance with one exemplary embodiment of the present invention four rollers with sand paper surfaces are used in order to treat the fabric. However, it is to be understood that any number of rollers can be used in other embodiments and that their surfaces need not be rough. In one embodiment, the fabric is passed over a first roller that rotates in a first direction and has a 120 grit sand paper surface. The first roller presses onto the fabric surface in order to cause 3 inches of compression thereto.

A second roller can be employed and may have a 100 grit sand paper surface. The second roller can rotate in a direction opposite to the first roller and may be tensioned against the fabric so as to cause 7 inches of compression thereto. A third roller may also be employed and can have a 100 grit sand paper surface. The third roller may, as with the second roller, rotate in a second direction. The third roller is tensioned against the fabric in order to cause 7 inches of compression. The fabric may also be passed over a fourth roller that has a 120 grit sand paper surface. The fourth roller, like the first roller, rotates in the first direction. The fourth roller is configured in order to be urged against the fabric so as to cause 5 inches of compression thereto.

The first direction that the first and fourth rollers rotate may be the counter clockwise direction. The second direction in which the second and third rollers rotate can be opposite that of the first direction and may be in the clockwise direction. In other versions of the present invention, the first, second, third and fourth rollers may rotate in directions other than those disclosed above. The rollers can be driven so they urge the fabric in the machine direction. Alternatively, the rollers can be free turning so they do not act to urge the fabric in the machine direction. In other configurations, some of the rollers may be driven while others are free turning. Further, although described as having sand paper surfaces, the rollers need not actually have sand paper applied thereto. Instead, the surfaces of the rollers may be rough so as to result in possessing a grit quality much like a piece of sand paper. Although described as imparting a certain amount of compression onto the fabric, the rollers may apply various amount of compression in other embodiments. Additionally, one or more of the rollers need not apply any amount of compression in other versions of the disclosed method.

Heretofore, efforts to sand large width fabrics, defined here as fabrics having a width equal to or in excess of 102 inches have not been commercially viable. Variations in the tension of the fabric and uniformity of the sanding rollers results in uneven areas of the fabric. It has been found that in accordance with the present invention using an exemplary fabric as described above, including fabrics which have been dyed or treated with fire retardant coatings, a large width fabric, such

as a 124 inch width fabric can be sanded to result in a fabric having a high quality hand with a uniform finish from edge to edge.

After sanding, the fabric is placed on a tenter frame and stretched a certain percentage of the fabric's relaxed length. For example, the fabric may be stretched 2% of the fabric's relaxed length. The fabric may be stretched along its width. As previously mentioned, the lengthwise direction of the fabric is in the same direction in which the warp yarns extend and is in the same direction as the machine direction of the rollers. The width of the fabric is perpendicular to the lengthwise direction of the fabric and is in the same direction as that in which the weft yarns extend.

In the disclosed method, the fabric can be treated once the fabric is applied to the tenter frame. For example, an agent may be applied to the fabric in order to improve various properties of the fabric such as soil release and pilling. In accordance with one exemplary embodiment, a chemical agent such as 2% LUBRIL® can be applied to the fabric after the fabric is applied to the tenter frame in order to improve soil release and improve pilling properties of the fabric. 2% LUBRIL® is distributed by Resolution Specialty Materials having offices located at 200 Railroad Street, Roebuck, S.C. 29376. The soil release property of the fabric relates to the ease with which dirt and other unwanted particles can be removed from the fabric upon washing. When used in items such as clothing and curtains, it is desirable for the article to easily release dirt contained thereon during cleaning. The pilling property of the fabric relates to the tendency of fibers of the fabric to interlock or knot with one another so as to form clumps on the surface of the fabric. Again, it is usually desirable for fabric used in applications such as clothing and curtains to have a minimum of pilling. Although described as being used in order to improve the soil release and pilling properties of fabric, it is to be understood that in other embodiments different types of agents may be applied to the fabric in order to modify other properties of the fabric.

While on the tenter frame, the fabric may be moved at a speed from 15 to 35 yards per minute. Other speeds are possible in other versions of the method. For example, the fabric may be moved at speeds up to 75 yards per minute in other embodiments.

The fabric is also heated to a temperature of 385 degrees Fahrenheit during application of the agent to the fabric. Heating of the fabric during application of the agent may act to impart durability and optimize performance of the agent. In other embodiments, the fabric may be heated before, after and/or during application of the agent. Further, the temperature to which the fabric is heated may vary. For example, the fabric may be heated to a temperature of from 380-420 degrees Fahrenheit. The tenter frame holds the fabric and maintains its stretch so that when dried the fabric does not shrink.

By employing rollers and a tenter frame that have elongated widths, the fabric is capable of being formed so that its width is about 124 inches. As such, the fabric can be formed with a desired width for a particular application without the need to sew two or more pieces of fabric together to achieve the desired width. This ability may be advantageous in that print patterns on two or more pieces of fabric do not need to be aligned with one another in forming a resultant fabric with a desired width. Further, as the fabric can be made to have a desired width the fabric can also be made without the presence of seams.

FIG. 1 shows a fabric 10 in accordance with one embodiment of the present invention. The fabric 10 can be used in constructing a wide variety of articles. For example, fabric 10

may be incorporated into curtains, clothing and/or covers. As shown, the fabric 10 has a longitudinal direction 12 that is perpendicular to the width 14 of the fabric 10. The longitudinal direction 12 may be in the same direction as is the machine direction during construction of the fabric 10. The width 14 is at least 102 inches and may be 124 inches in one embodiment. The face 16 of the fabric 10 is typically flat, lustrous and smooth and the fabric 10 is constructed with a twill weave with a satin face. The face 16 may be a relatively shiny surface if the yarns making up the fabric 10 are smooth and shiny. The weave pattern of yarns making up the fabric 10 may cause the face 16 to have different properties than the backside. However, the backside 18 may be treated the same as or differently from the face 16 so that properties of both the face 16 and backside 18, such as hand and shininess, may be the same as one another or different.

FIG. 2 is an enlarged view of the weave pattern noted in circle A of FIG. 1. The warp yarns 20 are arranged substantially parallel to one another and extend in the longitudinal direction 12 of fabric 10. The warp yarns 20 are arranged in such a pattern so as to lay over four weft yarns 22 and then under one weft yarn 22. The weft yarns 22 are oriented substantially parallel to one another and extend in the width 14 direction of fabric 20. As shown, the warp yarns 20 are arranged in a perpendicular fashion to the weft yarns 22. The weave pattern shown in FIG. 2 may repeat throughout the rest of fabric 10 and is known as a 4/1 twill weave with a satin face. The float of fabric 10 is 4/1 because the warp yarn 20 overlays four weft yarns 22 before laying under one weft yarn 22.

FIG. 3 shows an alternative exemplary embodiment of the fabric 10 in accordance with the present invention that displays the weave pattern of fabric 10. As with the embodiment in FIG. 2, the warp yarns 20 are parallel to one another and oriented in the longitudinal direction 12. The weft yarns 22 are likewise parallel to one another and are oriented in the direction of the width 14 of fabric 10. In this embodiment, the warp yarns 20 are arranged so as to lay over three weft yarns 22 and then under one weft yarn 22. The weave pattern shown in FIG. 3 may repeat through the entire fabric 10 and is known as a 3/1 twill weave with a satin face.

Twill weave fabrics with a satin face generally have fewer interlacings and allow for more yarns per square inch to be used. These types of weaves also normally result in fabrics with better hand properties, more wrinkle resistance, more soil resistance, and more durability than plain weave fabrics. Also, twill weave fabrics with a satin face tend to have a more defined face and backside.

While the present invention has been described in connection with certain preferred embodiments, it is to be understood that the subject matter encompassed by way of the present invention is not to be limited to those specific embodiments. On the contrary, it is intended for the subject matter of the invention to include all alternatives, modifications and equivalents as can be included within the spirit and scope of the following claims.

#### Experiments Carried Out in Accordance with Various Exemplary Embodiments of the Present Invention

Experiments were conducted in accordance with various exemplary embodiments of the present invention. One such experiment measured the amount of pilling of the fabric. Pilling of the fabric involves the formation of fuzz balls on the face of the fabric that are formed by abrasion. A rating system is used in order to evaluate the pilling properties of a particular fabric:

| Rating of Pilling | Description of Pilling |
|-------------------|------------------------|
| Class 5           | No Pilling             |
| Class 4           | Slight Pilling         |
| Class 3           | Moderate Pilling       |
| Class 2           | Severe Pilling         |
| Class 1           | Very Severe Pilling    |

Several specimens were tested to evaluate pilling properties as per an ASTM D 3512 testing procedure which is a standard test method for pilling resistance and other related surface changes of textile fabrics. This test method is sometimes known as a random tumble filling tester method. The specimens were treated in a manner as disclosed in the present application. The results were as follows:

| Specimen | Rating After 30 Minutes |
|----------|-------------------------|
| 1        | Class 5*                |
| 2        | Class 5*                |
| 3        | Class 5*                |

Although the 3 specimens tested that were made in accordance with the present invention rated as a class 5, they were found to have a slight degree of fuzzing of their outer surface.

Additional experiments were carried out on fabrics produced in accordance with the method of the present application. Further experiments were directed towards evaluating the wetting property of the fabric. Wetting is a test of the ability of water or another cleaning liquid to pass through the fabric. A rating system was used to evaluate the property of wetting:

| Wetting Score | Description                                        |
|---------------|----------------------------------------------------|
| 100           | No Sticking or Wetting of Upper Surface            |
| 90            | Slight Random Sticking or Wetting of Upper Surface |
| 80            | Wetting of Upper Surface at Spray Points           |
| 70            | Partial Wetting of Whole of Upper Surface          |
| 50            | Complete Wetting of Whole of Upper Surface         |
| 0             | Complete Wetting of Whole Upper and Lower Surfaces |

A spray test was performed using an AATCC test method 22. Here, water was sprayed against a taut surface of the test specimen under controlled conditions to produce a wetted pattern. The wetted pattern was compared with pictures on a standard chart in order to accomplish the evaluation. The results were as follows:

| Specimen | Rating |
|----------|--------|
| 1        | 0      |
| 2        | 0      |
| 3        | 0      |

The wetting properties of fabric made in accordance with the present invention were found to have a wetting score of 0.

An additional experiment was carried out on fabric made in accordance with the present invention to determine fire retardance of the fabric. The test performed was an NFPA 701-2004 TM#1 which is a 2004 edition standard fire test for flame propagation of textiles and films. The minimum requirement

for contract drapery is the NFPA 701 testing method. The fabric tested was configured as a single layer and the test results on the fabric were reported immediately after the flame test was conducted so that the fabric was not laundered before its evaluation. The test results were as follows:

| Specimen | Afterflame* | Flaming Drip | Weight Loss | Flame projects<br>Above Top of<br>Specimen<br>(yes/no) | 10        |            |
|----------|-------------|--------------|-------------|--------------------------------------------------------|-----------|------------|
|          |             |              |             |                                                        | Mean: 1.5 | Mean: 22.3 |
| 1        | 0.0         | 0.0          | 24.1        | No                                                     |           |            |
| 2        | 29.7        | 10.0         | 18.3        | No                                                     |           |            |
| 3        | 14.1        | 2.3          | 25.2        | No                                                     |           |            |
| 4        | 0.0         | 0.0          | 24.8        | No                                                     |           |            |
| 5        | 0.0         | 0.0          | 24.5        | No                                                     |           |            |
| 6        | 10.5        | 0.0          | 31.2        | No                                                     |           |            |
| 7        | 0.0         | 2.3          | 29.5        | No                                                     |           |            |
| 8        | 0.0         | 0.0          | 17.3        | No                                                     |           |            |
| 9        | 0.0         | 0.0          | 14.8        | No                                                     |           |            |
| 10       | 0.0         | 0.0          | 13.1        | No                                                     |           |            |

The weight loss had a standard deviation (SD) of 6.1 so that  $3 \times SD = 18.3$ . The Mean + (3  $\times$  SD) = 40.6. The approximate weight of the material was measured to be  $219 \text{ g/m}^2$ . The specimens were prepared in the length direction and were preconditioned for a length of time of 30 minutes at a temperature of  $220^\circ \text{ F}$ . A conversion factor of  $\text{g/m}^2 + 28.35 \times 0.835 = \text{oz/yd}^2$  was used.

Failure criteria under the selected test method is as follows:

| 35                    |                   |             |                     |
|-----------------------|-------------------|-------------|---------------------|
| Weight Loss (percent) |                   |             |                     |
| Afterflame            | Flaming Drip      | Mean        | Individual Specimen |
| *                     | Exceeds 2 seconds | Exceeds 40% | Exceeds Mean + 3 SD |

Based on the failure criteria, the tested specimens pass the NFPA 701-2004 Edition test.

A revised failure criteria was also considered as follows:

| Afterflame | Mean              | Flaming Drip | Weight Loss |                                | Flame Height<br>(Individual Specimen) |
|------------|-------------------|--------------|-------------|--------------------------------|---------------------------------------|
|            |                   |              | Mean        | Ind. Spec.                     |                                       |
| *          | Exceeds 2 seconds | Exceeds 40%  | Exceeds 50% | Projects above top of specimen |                                       |

In a similar manner, the specimens pass under the revised failure criteria. Although the NFPA document does not factor afterflame into the failure criteria reporting requirements, afterflame is recorded. It should be noted that excessive afterflame (15 seconds or more) may be cause for rejection of the product by local fire authorities performing "match" field tests.

Another test was carried out on fabric produced in accordance with the present invention to determine tearing strength. The test used was the ASTM D 2261 test which is a standard test method for tearing strength of fabrics by the tongue (single rip) procedure. The type of machine used in the test is a constant rate of extension tensile testing machine. Results of the test are as follows:

| Specimen # | Strength Across Warp (lbs) |              | Strength Across Fill (lbs) |
|------------|----------------------------|--------------|----------------------------|
|            | 5                          | 10           |                            |
| 1          | 30.5                       | Average 29.9 | 27.5                       |
| 2          | 31.0                       |              | 29.0                       |
| 3          | 33.5                       |              | 31.5                       |
| 4          | 27.5                       |              | 32.0                       |
| 5          | 27.0                       |              | 32.5                       |
|            |                            | Average 30.5 |                            |

Additional experiments were carried out in order to determine the breaking force of the fabric. The test method employed was the ASTM D 5034 test method that is sometimes known as the grab test and is a standard test method for measuring the breaking force of textile fabrics. The results of this test are as follows:

| Direction | Specimen # | Force (lbs) |
|-----------|------------|-------------|
| Warp      | 1          | 210         |
|           | 2          | 210         |
|           | 3          | 212         |
|           | 4          | 214         |
|           | 5          | 220         |
|           |            | Average 213 |
|           | 1          | 206         |
|           | 2          | 222         |
|           | 3          | 208         |
|           | 4          | 228         |
| Fill      | 5          | 224         |
|           | 6          | 240         |
|           | 7          | 242         |
|           | 8          | 247         |
|           |            | Average 227 |

Additional testing of the fabric was conducted. This additional test was the AATCC test method 135 that ascertained dimensional changes in automatic home laundering of woven and knit fabrics. The fabric was subjected to both one and five laundering cycles and a wash load of four pounds was used. The washing machine used was set at a normal/ctn/sturdy setting with a wash temperature of  $160^\circ \text{ F} \pm 5^\circ \text{ F}$  with a tumble dry of cotton/sturdy. The results are as follows (- indicating shrinkage and + indicating growth):

| 50            | Results after 1 cycle |                     | Results after 2 cycles |                     |
|---------------|-----------------------|---------------------|------------------------|---------------------|
|               | (% change)<br>Length  | (% change)<br>Width | (% change)<br>Length   | (% change)<br>Width |
| -0.5          | 0.0                   | -0.5                | 0.0                    |                     |
| -0.5          | 0.0                   | -0.5                | 0.0                    |                     |
| -0.5          | 0.0                   | -0.5                | 0.0                    |                     |
| Average: -0.5 | Average 0.0           | Average -0.5        | Average 0.0            |                     |

The ASTM D 4157-02 test was also conducted which is a standard test method for measuring abrasion resistance of textile fabrics and is sometimes known as an oscillatory cylinder method. Wire (steel) screen was selected as an abradant. The surface category into which the fabric falls is a special surface effect which is used for napped, chenille, embossed, textured and like fabrics. The specimen was tensioned at 4 pounds and a head pressure of 3 pounds was applied. The rating system special surface effects are as follows:

## 11

- 5—None or negligible wear/change of special surface effect  
 4—Slight wear/change of special surface effect  
 3—Moderate wear/change of special surface effect  
 2—Noticeable wear/change of special surface effect (base  
 10      yarns exposed)  
 1—Severe wear/change of special surface effect (base  
      yarns exposed and broken)  
 The test results obtained through visible observations are  
 as follows:

| Number of Double Rubs | Length Specimens                          | Width Specimens                           |
|-----------------------|-------------------------------------------|-------------------------------------------|
| 3,000                 | 4.5-5.0                                   | 4.5-5.0                                   |
| 9,000                 | 4.0                                       | 4.0                                       |
| 15,000                | 3.5-4.0                                   | 3.5-4.0                                   |
| 22,500                | 3.0-3.5                                   | 3.0-3.5                                   |
| 30,000                | 3.0 - Moderate loss of<br>surface texture | 3.0 - Moderate loss of<br>surface texture |

Class 3 is generally considered to be the minimum passing rate for heavy duty commercial upholstery. Light duty upholstery standards are typically 9,000 rubs with class 3 performance.

## What is claimed:

1. A method of finishing a fabric having a twill weave with a satin face, comprising the steps of:  
 providing a fabric having a width from 102 to 131 inches;  
 sewing and batching said fabric on an A-frame;  
 passing said fabric at a speed of 20 yards per minute with a  
 first roll having a 120 grit sand paper surface and rotating  
 in a counter clockwise direction, wherein said first roll  
 applies 3 inches of compression to said fabric;  
 engaging said fabric with a second roll having a 100 grit  
 sand paper surface and rotating in a clockwise direction,  
 wherein said second roll applies 7 inches of compression  
 to said fabric;  
 engaging said fabric with a third roll having a 100 grit sand  
 paper surface and rotating in a clockwise direction,  
 wherein said third roll applies 7 inches of compression  
 to said fabric;  
 engaging said fabric with a fourth roll having a 120 grit sand  
 paper surface and rotating in a counter clockwise direction,  
 wherein said fourth roll applies 5 inches of  
 compression to said fabric;  
 applying said fabric to a tenter frame;  
 stretching said fabric by 2% of said fabric's relaxed length;  
 moving said fabric at a speed from 15 to 35 yards per  
 minute; and  
 applying an agent to said fabric to improve pilling proper-  
 ties of said fabric;  
 heating said fabric to a temperature of 385 degrees Fahr-  
 enheit.
2. The method as in claim 1, wherein said fabric has a float  
 selected from the group consisting of 3/1 and 4/1.
3. A method of forming a fabric, comprising the steps of:  
 providing a plurality of yarn;  
 batching said yarn on an A-frame such that said fabric is  
 formed having a width greater than 102 inches and hav-  
 ing a twill weave with a satin face;  
 passing said fabric across a plurality of rolls that have a  
 rough surface, wherein said rolls apply compression to  
 said fabric;  
 applying said fabric to a tenter frame; and  
 heating said fabric.

## 12

4. The method as in claim 3, further comprising the step of  
 sanding said fabric at a speed of 20 yards per minute.
5. The method as in claim 3, wherein said passing step  
 comprising:  
 passing said fabric across a first roll having a 120 grit sand  
 paper surface and rotating in a first direction, wherein  
 said first roll applies at least 3 inches of compression to  
 said fabric;  
 passing said fabric across a second roll having a 100 grit  
 sand paper surface and rotating in a second direction,  
 wherein said second roll applies at least 7 inches of  
 compression to said fabric;  
 passing said fabric across a third roll having a 100 grit sand  
 paper surface and rotating in the second direction,  
 wherein said third roll applies at least 7 inches of com-  
 pression to said fabric; and  
 passing said fabric across a fourth roll having a 120 grit  
 sand paper surface and rotating in the first direction,  
 wherein said fourth roll applies at least 5 inches of com-  
 pression to said fabric.
6. The method as in claim 5, wherein the first direction is  
 counter clockwise and wherein the second direction is clock-  
 wise.
7. The method as in claim 3, wherein said applying step  
 comprising stretching said fabric by 2% of said fabric's  
 relaxed length.
8. The method as in claim 3, further comprising the step of  
 applying an agent to said fabric to improve soil release and  
 pilling properties of said fabric.
9. The method as in claim 3, wherein after said batching  
 step said fabric is moved at a speed from 15 to 35 yards per  
 minute.
10. The method as in claim 3, wherein said heating step is  
 performed such that said fabric is heated to a temperature of  
 385 degree Fahrenheit.
11. The method as in claim 3, wherein said fabric is formed  
 in said batching step so as to have a float of 3/1.
12. The method as in claim 3, wherein said fabric is formed  
 in said batching step so as to have a float of 4/1.
13. The method as in claim 3, wherein the width of said  
 fabric is 124 inches.
14. A method of forming a fabric, comprising the steps of:  
 providing a plurality of polyester yarn;  
 sewing and batching said yarn on an A-frame such that said  
 fabric is formed having a width from 102 inches to 131  
 inches and having a 3/1 or 4/1 twill weave with a satin  
 face;  
 sanding said fabric at a speed of at least 20 yards per  
 minute;
- 55
- passing said fabric across a plurality of rolls that have a  
 sand paper surface, wherein said rolls apply compres-  
 sion to said fabric;
- applying said fabric to a tenter frame such that said fabric  
 is stretched by at least 2% of said fabric's relaxed length;  
 treating said fabric with an agent to improve pilling prop-  
 60  
 65  
 70  
 75  
 80  
 85  
 90  
 95  
 100  
 105  
 110  
 115  
 120  
 125  
 130  
 135  
 140  
 145  
 150  
 155  
 160  
 165  
 170  
 175  
 180  
 185  
 190  
 195  
 200  
 205  
 210  
 215  
 220  
 225  
 230  
 235  
 240  
 245  
 250  
 255  
 260  
 265  
 270  
 275  
 280  
 285  
 290  
 295  
 300  
 305  
 310  
 315  
 320  
 325  
 330  
 335  
 340  
 345  
 350  
 355  
 360  
 365  
 370  
 375  
 380  
 385  
 390  
 395  
 400  
 405  
 410  
 415  
 420  
 425  
 430  
 435  
 440  
 445  
 450  
 455  
 460  
 465  
 470  
 475  
 480  
 485  
 490  
 495  
 500  
 505  
 510  
 515  
 520  
 525  
 530  
 535  
 540  
 545  
 550  
 555  
 560  
 565  
 570  
 575  
 580  
 585  
 590  
 595  
 600  
 605  
 610  
 615  
 620  
 625  
 630  
 635  
 640  
 645  
 650  
 655  
 660  
 665  
 670  
 675  
 680  
 685  
 690  
 695  
 700  
 705  
 710  
 715  
 720  
 725  
 730  
 735  
 740  
 745  
 750  
 755  
 760  
 765  
 770  
 775  
 780  
 785  
 790  
 795  
 800  
 805  
 810  
 815  
 820  
 825  
 830  
 835  
 840  
 845  
 850  
 855  
 860  
 865  
 870  
 875  
 880  
 885  
 890  
 895  
 900  
 905  
 910  
 915  
 920  
 925  
 930  
 935  
 940  
 945  
 950  
 955  
 960  
 965  
 970  
 975  
 980  
 985  
 990  
 995  
 1000  
 1005  
 1010  
 1015  
 1020  
 1025  
 1030  
 1035  
 1040  
 1045  
 1050  
 1055  
 1060  
 1065  
 1070  
 1075  
 1080  
 1085  
 1090  
 1095  
 1100  
 1105  
 1110  
 1115  
 1120  
 1125  
 1130  
 1135  
 1140  
 1145  
 1150  
 1155  
 1160  
 1165  
 1170  
 1175  
 1180  
 1185  
 1190  
 1195  
 1200  
 1205  
 1210  
 1215  
 1220  
 1225  
 1230  
 1235  
 1240  
 1245  
 1250  
 1255  
 1260  
 1265  
 1270  
 1275  
 1280  
 1285  
 1290  
 1295  
 1300  
 1305  
 1310  
 1315  
 1320  
 1325  
 1330  
 1335  
 1340  
 1345  
 1350  
 1355  
 1360  
 1365  
 1370  
 1375  
 1380  
 1385  
 1390  
 1395  
 1400  
 1405  
 1410  
 1415  
 1420  
 1425  
 1430  
 1435  
 1440  
 1445  
 1450  
 1455  
 1460  
 1465  
 1470  
 1475  
 1480  
 1485  
 1490  
 1495  
 1500  
 1505  
 1510  
 1515  
 1520  
 1525  
 1530  
 1535  
 1540  
 1545  
 1550  
 1555  
 1560  
 1565  
 1570  
 1575  
 1580  
 1585  
 1590  
 1595  
 1600  
 1605  
 1610  
 1615  
 1620  
 1625  
 1630  
 1635  
 1640  
 1645  
 1650  
 1655  
 1660  
 1665  
 1670  
 1675  
 1680  
 1685  
 1690  
 1695  
 1700  
 1705  
 1710  
 1715  
 1720  
 1725  
 1730  
 1735  
 1740  
 1745  
 1750  
 1755  
 1760  
 1765  
 1770  
 1775  
 1780  
 1785  
 1790  
 1795  
 1800  
 1805  
 1810  
 1815  
 1820  
 1825  
 1830  
 1835  
 1840  
 1845  
 1850  
 1855  
 1860  
 1865  
 1870  
 1875  
 1880  
 1885  
 1890  
 1895  
 1900  
 1905  
 1910  
 1915  
 1920  
 1925  
 1930  
 1935  
 1940  
 1945  
 1950  
 1955  
 1960  
 1965  
 1970  
 1975  
 1980  
 1985  
 1990  
 1995  
 2000  
 2005  
 2010  
 2015  
 2020  
 2025  
 2030  
 2035  
 2040  
 2045  
 2050  
 2055  
 2060  
 2065  
 2070  
 2075  
 2080  
 2085  
 2090  
 2095  
 2100  
 2105  
 2110  
 2115  
 2120  
 2125  
 2130  
 2135  
 2140  
 2145  
 2150  
 2155  
 2160  
 2165  
 2170  
 2175  
 2180  
 2185  
 2190  
 2195  
 2200  
 2205  
 2210  
 2215  
 2220  
 2225  
 2230  
 2235  
 2240  
 2245  
 2250  
 2255  
 2260  
 2265  
 2270  
 2275  
 2280  
 2285  
 2290  
 2295  
 2300  
 2305  
 2310  
 2315  
 2320  
 2325  
 2330  
 2335  
 2340  
 2345  
 2350  
 2355  
 2360  
 2365  
 2370  
 2375  
 2380  
 2385  
 2390  
 2395  
 2400  
 2405  
 2410  
 2415  
 2420  
 2425  
 2430  
 2435  
 2440  
 2445  
 2450  
 2455  
 2460  
 2465  
 2470  
 2475  
 2480  
 2485  
 2490  
 2495  
 2500  
 2505  
 2510  
 2515  
 2520  
 2525  
 2530  
 2535  
 2540  
 2545  
 2550  
 2555  
 2560  
 2565  
 2570  
 2575  
 2580  
 2585  
 2590  
 2595  
 2600  
 2605  
 2610  
 2615  
 2620  
 2625  
 2630  
 2635  
 2640  
 2645  
 2650  
 2655  
 2660  
 2665  
 2670  
 2675  
 2680  
 2685  
 2690  
 2695  
 2700  
 2705  
 2710  
 2715  
 2720  
 2725  
 2730  
 2735  
 2740  
 2745  
 2750  
 2755  
 2760  
 2765  
 2770  
 2775  
 2780  
 2785  
 2790  
 2795  
 2800  
 2805  
 2810  
 2815  
 2820  
 2825  
 2830  
 2835  
 2840  
 2845  
 2850  
 2855  
 2860  
 2865  
 2870  
 2875  
 2880  
 2885  
 2890  
 2895  
 2900  
 2905  
 2910  
 2915  
 2920  
 2925  
 2930  
 2935  
 2940  
 2945  
 2950  
 2955  
 2960  
 2965  
 2970  
 2975  
 2980  
 2985  
 2990  
 2995  
 3000  
 3005  
 3010  
 3015  
 3020  
 3025  
 3030  
 3035  
 3040  
 3045  
 3050  
 3055  
 3060  
 3065  
 3070  
 3075  
 3080  
 3085  
 3090  
 3095  
 3100  
 3105  
 3110  
 3115  
 3120  
 3125  
 3130  
 3135  
 3140  
 3145  
 3150  
 3155  
 3160  
 3165  
 3170  
 3175  
 3180  
 3185  
 3190  
 3195  
 3200  
 3205  
 3210  
 3215  
 3220  
 3225  
 3230  
 3235  
 3240  
 3245  
 3250  
 3255  
 3260  
 3265  
 3270  
 3275  
 3280  
 3285  
 3290  
 3295  
 3300  
 3305  
 3310  
 3315  
 3320  
 3325  
 3330  
 3335  
 3340  
 3345  
 3350  
 3355  
 3360  
 3365  
 3370  
 3375  
 3380  
 3385  
 3390  
 3395  
 3400  
 3405  
 3410  
 3415  
 3420  
 3425  
 3430  
 3435  
 3440  
 3445  
 3450  
 3455  
 3460  
 3465  
 3470  
 3475  
 3480  
 3485  
 3490  
 3495  
 3500  
 3505  
 3510  
 3515  
 3520  
 3525  
 3530  
 3535  
 3540  
 3545  
 3550  
 3555  
 3560  
 3565  
 3570  
 3575  
 3580  
 3585  
 3590  
 3595  
 3600  
 3605  
 3610  
 3615  
 3620  
 3625  
 3630  
 3635  
 3640  
 3645  
 3650  
 3655  
 3660  
 3665  
 3670  
 3675  
 3680  
 3685  
 3690  
 3695  
 3700  
 3705  
 3710  
 3715  
 3720  
 3725  
 3730  
 3735  
 3740  
 3745  
 3750  
 3755  
 3760  
 3765  
 3770  
 3775  
 3780  
 3785  
 3790  
 3795  
 3800  
 3805  
 3810  
 3815  
 3820  
 3825  
 3830  
 3835  
 3840  
 3845  
 3850  
 3855  
 3860  
 3865  
 3870  
 3875  
 3880  
 3885  
 3890  
 3895  
 3900  
 3905  
 3910  
 3915  
 3920  
 3925  
 3930  
 3935  
 3940  
 3945  
 3950  
 3955  
 3960  
 3965  
 3970  
 3975  
 3980  
 3985  
 3990  
 3995  
 4000  
 4005  
 4010  
 4015  
 4020  
 4025  
 4030  
 4035  
 4040  
 4045  
 4050  
 4055  
 4060  
 4065  
 4070  
 4075  
 4080  
 4085  
 4090  
 4095  
 4100  
 4105  
 4110  
 4115  
 4120  
 4125  
 4130  
 4135  
 4140  
 4145  
 4150  
 4155  
 4160  
 4165  
 4170  
 4175  
 4180  
 4185  
 4190  
 4195  
 4200  
 4205  
 4210  
 4215  
 4220  
 4225  
 4230  
 4235  
 4240  
 4245  
 4250  
 4255  
 4260  
 4265  
 4270  
 4275  
 4280  
 4285  
 4290  
 4295  
 4300  
 4305  
 4310  
 4315  
 4320  
 4325  
 4330  
 4335  
 4340  
 4345  
 4350  
 4355  
 4360  
 4365  
 4370  
 4375  
 4380  
 4385  
 4390  
 4395  
 4400  
 4405  
 4410  
 4415  
 4420  
 4425  
 4430  
 4435  
 4440  
 4445  
 4450  
 4455  
 4460  
 4465  
 4470  
 4475  
 4480  
 4485  
 4490  
 4495  
 4500  
 4505  
 4510  
 4515  
 4520  
 4525  
 4530  
 4535  
 4540  
 4545  
 4550  
 4555  
 4560  
 4565  
 4570  
 4575  
 4580  
 4585  
 4590  
 4595  
 4600  
 4605  
 4610  
 4615  
 4620  
 4625  
 4630  
 4635  
 4640  
 4645  
 4650  
 4655  
 4660  
 4665  
 4670  
 4675  
 4680  
 4685  
 4690  
 4695  
 4700  
 4705  
 4710  
 4715  
 4720  
 4725  
 4730  
 4735  
 4740  
 4745  
 4750  
 4755  
 4760  
 4765  
 4770  
 4775  
 4780  
 4785  
 4790  
 4795  
 4800  
 4805  
 4810  
 4815  
 4820  
 4825  
 4830  
 4835  
 4840  
 4845  
 4850  
 4855  
 4860  
 4865  
 4870  
 4875  
 4880  
 4885  
 4890  
 4895  
 4900  
 4905  
 4910  
 4915  
 4920  
 4925  
 4930  
 4935  
 4940  
 4945  
 4950  
 4955  
 4960  
 4965  
 4970  
 4975  
 4980  
 4985  
 4990  
 4995  
 5000  
 5005  
 5010  
 5015  
 5020  
 5025  
 5030  
 5035  
 5040  
 5045  
 5050  
 5055  
 5060  
 5065  
 5070  
 5075  
 5080  
 5085  
 5090  
 5095  
 5100  
 5105  
 5110  
 5115  
 5120  
 5125  
 5130  
 5135  
 5140  
 5145  
 5150  
 5155  
 5160  
 5165  
 5170  
 5175  
 5180  
 5185  
 5190  
 5195  
 5200  
 5205  
 5210  
 5215  
 5220  
 5225  
 5230  
 5235  
 5240  
 5245  
 5250  
 5255  
 5260  
 5265  
 5270  
 5275  
 5280  
 5285  
 5290  
 5295  
 5300  
 5305  
 5310  
 5315  
 5320  
 5325  
 5330  
 5335  
 5340  
 5345  
 5350  
 5355  
 5360  
 5365  
 5370  
 5375  
 5380  
 5385  
 5390  
 5395  
 5400  
 5405  
 5410  
 5415  
 5420  
 5425  
 5430  
 5435  
 5440  
 5445  
 5450  
 5455  
 5460  
 5465  
 5470  
 5475  
 5480  
 5485  
 5490  
 5495  
 5500  
 5505  
 5510  
 5515  
 5520  
 5525  
 5530  
 5535  
 5540  
 5545  
 5550  
 5555  
 5560  
 5565  
 5570  
 5575  
 5580  
 5585  
 5590  
 5595  
 5600  
 5605  
 5610  
 5615  
 5620  
 5625  
 5630  
 5635  
 5640  
 5645  
 5650  
 5655  
 5660  
 5665  
 5670  
 5675  
 5680  
 5685  
 5690  
 5695  
 5700  
 5705  
 5710  
 5715  
 5720  
 5725  
 5730  
 5735  
 5740  
 5745  
 5750  
 5755  
 5760  
 5765  
 5770  
 5775  
 5780  
 5785  
 5790  
 5795  
 5800  
 5805  
 5810  
 5815  
 5820  
 5825  
 5830  
 5835  
 5840  
 5845  
 5850  
 5855  
 5860  
 5865  
 5870  
 5875  
 5880  
 5885  
 5890  
 5895

**13**

passing said fabric across a second roll having a 100 grit sand paper surface and rotating in a second direction, wherein said second roll applies at least 7 inches of compression to said fabric;

passing said fabric across a third roll having a 100 grit sand paper surface and rotating in the second direction, wherein said third roll applies at least 7 inches of compression to said fabric; and

**14**

passing said fabric across a fourth roll having a 120 grit sand paper surface and rotating in the first direction, wherein said fourth roll applies at least 5 inches of compression to said fabric.

5 **16.** The method as in claim **14**, further comprising the step of moving said fabric at a speed from 15 to 35 yards per minute.

\* \* \* \* \*